

## UNITED STATES PATENT OFFICE

AXEL VIGGO BLOM, OF GROSSHOECHSTETTEN, SWITZERLAND

## PROCESS FOR PRODUCING PIGMENTARY BASE PRODUCTS FOR LEAD PAINTS

No Drawing.

Application filed April 5, 1927. Serial No. 181,279.

My invention concerns a process for producing materials adapted to serve as pigmentary bases for paints and particularly lead paints suitable for use as rust proof coating for iron and other objects and surfaces. In my copending application, Serial No. 181,278, filed April 5, 1927, I have described a new and improved material of this character and a process suitable for producing the same. In carrying out the said process, I have found that the oxidation of the metallic lead or lead alloy as carried out in my process is occasionally somewhat sluggish. I have discovered that this sluggishness can be overcome and the reaction speeded up by the presence of catalyzing substances. I have also found that it is not necessary to use large quantities of catalyzing substances as compared to the quantity of material under treatment, but that even a comparatively small amount of the said catalysts is sufficient to show a decided influence on the speed of the reaction. As such catalyzing substance I have found that all the salts of calcium with high molecular organic acids are suitable, for example, the resinate, naphthenate, and oleate salts, but I preferably use calcium resinate and I have observed that as little as one-half per cent of this substance affects appreciably the speeding up of the oxidizing reaction. In carrying out my invention I proceed in the following manner.

I take metallic lead or an alloy containing a high percentage of lead such as described in my copending application, Serial No. 181,278, filed April 5, 1927, for instance an alloy containing 85% lead, 13% antimony and 2% tin, and melt the same in a furnace of the usual construction, provided with a flat pan-shaped hearth, in the presence of  $\frac{1}{2}$  per cent of calcium resinate. The interior of the said furnace is adapted to be closed air tight, so that a certain vacuum can be established therein. I then cause the said molten metal to undergo a slow oxidation process by means

of creating a vacuum in the interior of the said furnace and drawing air into the same from the outside through a plurality of tuyères located in a suitable position above the molten bath. The action of the air causes the slow oxidation of the molten bath and the formation of a pigmentary base of the character described in my copending application, mentioned above.

As the pigmentary body forms on the surface of the molten bath it is carried away by the suction of the air introduced into the furnace. It is collected in any suitable manner, such for instance in a bag plant similar to those used for the deposition of flue dust.

Having thus described my invention what I claim as new and desire to secure by Letters Patent is:—

1. A continuous process for producing a pigmentary base of the character described, which consists in melting a lead alloy containing a large percentage of lead in a thin layer in an air tight furnace in the presence of calcium resinate, establishing a vacuum in the said furnace, causing the said molten lead to be acted upon by a plurality of streams of air drawn into the said furnace by the vacuum, continuously removing the product and separating therefrom all particles larger than 50 microns.

2. A continuous process for producing a pigmentary base of the character described, which consists in melting a lead alloy containing a large percentage of lead in a thin layer in an air tight furnace in the presence of a small percentage of calcium resinate, establishing a vacuum in the said furnace, causing the said molten lead to be acted upon by a plurality of streams of air drawn into the said furnace by the vacuum, continuously removing the product and separating therefrom all particles larger than 50 microns.

3. A continuous process for producing a pigmentary base of the character described, which consists in melting an alloy composed

of 85 per cent lead, 13 per cent antimony, and 2 per cent tin in the presence of a small percentage of calcium resinate in a thin layer in an air tight furnace, establishing a vacuum in the said furnace, causing the said molten lead to be acted upon by a plurality of streams of air drawn into the said furnace by the vacuum, continuously removing the product and separating therefrom all particles larger than 50 microns.

10. In testimony whereof, I have signed my name to this specification this twenty-third day of February, 1927.

AXEL VIGGO BLOM.

15

20

25

30

35

40

45

50

55

60

65